



US011651880B2

(12) **United States Patent**  
**Yamashita**

(10) **Patent No.:** US 11,651,880 B2  
(45) **Date of Patent:** May 16, 2023

(54) **COMPOSITE PARTICLE, CORE, AND INDUCTOR ELEMENT**

(71) Applicant: **TDK CORPORATION**, Tokyo (JP)

(72) Inventor: **Yasuhide Yamashita**, Tokyo (JP)

(73) Assignee: **TDK CORPORATION**, Tokyo (JP)

(\*) Notice: Subject to any disclaimer, the term of this patent is extended or adjusted under 35 U.S.C. 154(b) by 369 days.

(21) Appl. No.: **16/827,950**

(22) Filed: **Mar. 24, 2020**

(65) **Prior Publication Data**

US 2020/0312502 A1 Oct. 1, 2020

(30) **Foreign Application Priority Data**

Mar. 27, 2019 (JP) ..... JP2019-060954

(51) **Int. Cl.**

**H01F 1/20** (2006.01)  
**H01F 1/147** (2006.01)  
**H01F 27/255** (2006.01)  
**H01F 17/04** (2006.01)  
**H01F 41/02** (2006.01)

(52) **U.S. Cl.**

CPC ..... **H01F 1/20** (2013.01); **H01F 1/14733** (2013.01); **H01F 1/14766** (2013.01); **H01F 17/04** (2013.01); **H01F 27/255** (2013.01); **H01F 41/0246** (2013.01); **Y10T 428/32** (2015.01)

(58) **Field of Classification Search**

None

See application file for complete search history.

(56) **References Cited**

U.S. PATENT DOCUMENTS

|                   |         |                 |
|-------------------|---------|-----------------|
| 6,136,265 A       | 10/2000 | Gay             |
| 10,410,774 B2 *   | 9/2019  | Kusawake .....  |
| 10,774,404 B2 *   | 9/2020  | Suetsuna .....  |
| 11,049,641 B2 *   | 6/2021  | Ohkubo .....    |
| 2014/0097377 A1 * | 4/2014  | Igarashi .....  |
|                   |         | B22F 5/006      |
|                   |         | 252/62.54       |
| 2014/0132383 A1   | 5/2014  | Matsuura et al. |
| 2016/0155550 A1 * | 6/2016  | Ohkubo .....    |
|                   |         | H01F 1/24       |
|                   |         | 336/233         |
| 2017/0209924 A1 * | 7/2017  | Suetsuna .....  |
| 2018/0043431 A1   | 2/2018  | Araki et al.    |
| 2018/0068771 A1 * | 3/2018  | Nakazawa .....  |
| 2018/0261385 A1 * | 9/2018  | Nakazawa .....  |
| 2019/0333666 A1 * | 10/2019 | Nakamura .....  |
| 2019/0392978 A1 * | 12/2019 | Matsuura .....  |
| 2020/0066437 A1 * | 2/2020  | Lee .....       |
| 2021/0053115 A1 * | 2/2021  | Takahashi ..... |
| 2021/0057139 A1 * | 2/2021  | Takahashi ..... |
| 2021/0129218 A1 * | 5/2021  | Matsumoto ..... |
| 2021/0183566 A1 * | 6/2021  | Ohkubo .....    |
| 2021/0304932 A1 * | 9/2021  | Yoshidome ..... |
|                   |         | C22C 45/02      |

(Continued)

FOREIGN PATENT DOCUMENTS

|    |               |        |
|----|---------------|--------|
| CN | 108364766 A   | 8/2018 |
| JP | 2005-243769 A | 9/2005 |

(Continued)

*Primary Examiner* — Kevin M Bernatz

(74) *Attorney, Agent, or Firm* — Oliff PLC

(57) **ABSTRACT**

A composite particle includes a large particle and binder particles. The large particle has a particle size of 10  $\mu\text{m}$  to 50  $\mu\text{m}$ . The binder particles are attached on the large particle and each have a particle size smaller than that of the large particle.

**12 Claims, 5 Drawing Sheets**



(56)

**References Cited**

U.S. PATENT DOCUMENTS

2021/0335526 A1\* 10/2021 Yamashita ..... H01F 1/344  
2021/0391112 A1\* 12/2021 Yamashita ..... H01F 1/24

FOREIGN PATENT DOCUMENTS

JP 2016-180154 A 10/2016  
JP 2018-152557 A 9/2018  
WO 2012/147576 A1 11/2012

\* cited by examiner

FIG. 1



FIG. 2



FIG. 3



FIG. 4



FIG. 5



## 1

COMPOSITE PARTICLE, CORE, AND  
INDUCTOR ELEMENT

## BACKGROUND OF THE INVENTION

The present invention relates to a composite particle, such as a composite particle constituting a core.

As described in Patent Document 1, widely used as a coil-type electronic component is a core obtained by putting metal magnetic particles and a binder into a predetermined die and pressing them.

However, it is difficult to disperse the binder to the metal magnetic particles. As a result, the coil-type electronic component has a problem with characteristic variation after pressing.

Patent Document 1: WO2012147576 (A1)

## BRIEF SUMMARY OF INVENTION

The present invention has been achieved under the above-mentioned problem. It is an object of the invention to provide composite particles with less characteristic variation after pressing and a core and an inductor element using the composite particles.

That is, an embodiment of the present invention is as follows.

[1] A composite particle includes:

a large particle having a particle size of 10  $\mu\text{m}$  to 50  $\mu\text{m}$ ; and

binder particles attached on the large particle and each having a particle size smaller than that of the large particle.

[2] The composite particle according to [1] further includes two or more small particles attached on the large particle and each having a particle size smaller than that of the large particle,

wherein at least one of the binder particles is attached on the large particle and located between two small particles among the two or more small particles attached on the large particle.

[3] The composite particle according to [2], wherein the small particles are magnetic particles.

[4] The composite particle according to any of [1] to [3], wherein the large particle is a magnetic particle.

[5] The composite particle according to any of [2] to [4], wherein each of the binder particles has a particle size smaller than that of the small particles.

[6] The composite particle according to any of [1] to [5], wherein the binder particles are deposited and attached on the large particle.

[7] A core has a cross section or a surface on which the composite particle according to any of [1] to [6] is observed.

[8] An inductor element includes the core according to [7].

[9] A method of manufacturing composite particles includes the steps of:

preparing a first solution in which large particles each having a particle size of 10  $\mu\text{m}$  to 50  $\mu\text{m}$  are dispersed in a binder soluble solution in which a binder is dissolved;

preparing a second solution in which a binder insoluble solution is added to the first solution; and

drying the second solution,

wherein the binder soluble solution is soluble to the binder and the binder insoluble solution, and

wherein the binder insoluble solution is insoluble to the binder.

[10] The method according to [9], wherein an aggregation inhibitor is added to the first solution in preparing the second solution.

## 2

[11] The method according to [9] or [10], wherein a small particle having a particle size smaller than that of each of the large particles is attached on each of the large particles in the first solution.

[12] Composite particles are obtained by the method according to any of [9] to [11].

## BRIEF DESCRIPTION OF DRAWINGS

10 FIG. 1 is a cross-sectional view of an inductor element according to an embodiment of the present invention.

FIG. 2 is a schematic cross-sectional view of a composite particle according to an embodiment of the present invention.

15 FIG. 3 is a schematic cross-sectional view of composite particles according to an embodiment of the present invention.

FIG. 4 is a schematic cross-sectional view of granules according to a comparative example of the present invention.

20 FIG. 5 is a graph relating to Examples 1-4 and Comparative Examples 1-4 of the present invention.

## DETAILED DESCRIPTION OF INVENTION

## 1. Inductor Element

As shown in FIG. 1, an inductor element 2 according to an embodiment of the present invention includes a winding part 4 and a core 6. A conductor 5 is wound in coil manner in the winding part 4. The core 6 is formed from particles and a binder.

For example, the core 6 is formed by pressing the particles and the binder. The particles are united with the binder, and the core 6 thereby has a predetermined fixed shape.

In the present embodiment, the particles and the binder constituting the core 6 are at least partly formed from, for example, predetermined composite particles 12 shown in FIG. 2.

Preferably, the ratio of the predetermined composite particles 12 shown in FIG. 2 to the total of the particles and the binder constituting the core 6 (100 mass %) is 93 mass % to 99.5 mass %. This makes it possible to obtain the following effects (“less characteristic variation after pressing” and “high consistency between pressing pressure and withstand voltage of the core 6 after pressing”) of the composite particles 12 according to the present embodiment.

## 1-1. Composite Particles

In each of the composite particles 12 according to the present embodiment, as shown in FIG. 2, small particles 18 and binder particles 16 are attached on a large particle 14. The large particle 14 has a particle size of 10  $\mu\text{m}$  to 50  $\mu\text{m}$  (preferably, 10  $\mu\text{m}$  to 25  $\mu\text{m}$ ).

In the present embodiment, the binder particles 16 are attached on each of the large particles 14 and each located between two small particles 18a and 18b among the small particles 18 attached on each of the large particles 14.

Here, “the binder particles 16 are attached on each of the large particles 14 and each located between two small particles 18a and 18b among the small particles 18 attached on each of the large particles 14” means that the binder particles 16 are attached on each of the large particles 14 and each located between connection points 38a and 38b of the two adjacent small particles 18a and 18b and each of the large particles 14.

Although explained below, each of the large particles 14 shown in FIG. 1 may include a cover part 24, and the small

particles **18a** and **18b** may also include a cover part **28**. In this case, strictly speaking, the connection point **38a** between the small particle **18a** and the large particle **14** mentioned above thereby means the connection point **38a** between the cover part **28a** of the small particle **18a** and the cover part **24** of the large particle **14**, and the connection point **38b** between the small particle **18b** and the large particle **14** thereby means the connection point **38b** between the cover part **28b** of the small particle **18b** and the cover part **24** of the large particle **14**.

The number of binder particles **16** attached on each of the large particles **14** and each located between the two small particles **18a** and **18b** attached on each of the large particles **14** is not limited, but is preferably one or more (more preferably, six or more). This makes it possible to obtain the composite particles **12** where the binder particles **16** are dispersed for each of the large particles **14**.

The particle size of the binder particles **16** attached on each of the large particles **14** and each located between the two small particles **18a** and **18b** attached on each of the large particle **14** is not limited, but is smaller than that of each of the large particles **14** and each of the small particles **18** and is preferably 0.1  $\mu\text{m}$  to 10  $\mu\text{m}$  (more preferably, 1  $\mu\text{m}$  to 7.5  $\mu\text{m}$ ). This makes it possible to obtain the composite particles **12** where the binder particles **16** are dispersed for each of the large particles **14**.

The number of small particles **18** attached on each of the large particles **14** is not limited, but is six or more, for example.

Preferably, each of  $(dL/dS)$ ,  $(dL/dB)$ , and  $(dS/dB)$  satisfies the following relation, where  $dL$  is a particle size of the large particle **14**,  $dS$  is a particle size of the small particle **18** attached on the large particle **14**, and  $dB$  is a particle size of the binder particle **16** attached on the large particle **14**.

That is, preferably,  $1 \leq (dL/dS) \leq 25$ . More preferably,  $1.4 \leq (dL/dS) \leq 8.3$ .

Preferably,  $1 \leq (dL/dB) \leq 500$ . More preferably,  $2 \leq (dL/dB) \leq 25$ .

Preferably,  $0.6 \leq (dS/dB) \leq 200$ . More preferably,  $1.0 \leq (dS/dB) \leq 7.0$ .

Incidentally, two or more composite particles **12** may aggregate as shown in FIG. 3.

The core **6** may conventionally be obtained by mixing a binder solution and the large particles **14** attached with the small particles **18**, volatilizing the binder solution without depositing binder particles, and pressing these granules. Instead, the core **6** may conventionally be obtained by spraying a binder solution against the large particles **14** attached with the small particles **18**, volatilizing the solvent of the binder solution, and pressing these granules.

In these granules, however, as shown in FIG. 4, a binder **46** unevenly unites the large particles **14** and the small particles **18** and is uneven in thickness among the particles and is not dispersively attached on the large particles **14**.

In these granules, the small particles **18** may aggregate and separate from the large particles **14** due to attraction of the small particles **18** by the binder **46**. As a result, the arrangement of the large particles **14** and the small particles **18** may change, and there is a problem with difficulty in obtaining desired characteristics.

On the other hand, since the composite particles **12** according to the present embodiment have the above-mentioned structure, the small particles **18** and the binder particles **16** are dispersively attached on the large particles **14**.

In the core **6** manufactured using the composite particles **12** according to the present embodiment, the binder is

uniformly present for the large particles **14** and the small particles **18**. Thus, the core **6** manufactured using the composite particles **12** according to the present embodiment has less characteristic variation after pressing.

In the manufacture of the core **6** using the composite particles **12** according to the present embodiment, there is a high consistency between pressing pressure and withstand voltage of the core **6** after pressing. Specifically, the higher pressing pressure is, the higher withstand voltage is. Thus, when the consistency between pressing pressure and withstand voltage is high, it is possible to obtain a desired withstand voltage based on pressing pressure and to stably adjust withstand voltage characteristics (product characteristics).

#### 1-1-1. Large Particles

In the present embodiment, the large particles **14** are magnetic particles. The inductor element **2** can be obtained by manufacturing the core **6** using the large particles **14**.

The magnetic particles of the large particles **14** are preferably metal magnetic particles or ferrite particles, more preferably metal magnetic particles. Still more preferably, the magnetic particles of the large particles **14** contain Fe.

Specifically, the metal magnetic particles containing Fe are pure iron, carbonyl Fe, Fe based alloy, Fe—Si based alloy, Fe—Al based alloy, Fe—Ni based alloy, Fe—Si—Al based alloy, Fe—Si—Cr based alloy, Fe—Co based alloy, Fe based amorphous alloy, Fe based nanocrystalline alloy, etc. Preferably, the metal magnetic particles containing Fe are Fe—Si based alloy.

The ferrite particles are Mn—Zn, Ni—Cu—Zn, etc.

In the present embodiment, the large particles **14** may be structured by a plurality of large particles composed of the same material or a plurality of mixed large particles composed of different materials. For example, multiple Fe based alloy particles and multiple Fe—Si based alloy particles may be mixed and used for the large particles **14**.

Each of the large particles **14** according to the present embodiment has a particle size of 10  $\mu\text{m}$  to 50  $\mu\text{m}$  (preferably, 20  $\mu\text{m}$  to 25  $\mu\text{m}$ ).

Incidentally, the above-mentioned particle size excludes the cover part **24** of each of the large particles **14** mentioned below.

When the large particles **14** are structured by large particles composed of two or more types of different materials, the large particles composed of a certain material and the large particles composed of another material may have different particle sizes.

Incidentally, for example, the different materials mean that elements constituting metal or alloy are different from each other or that elements constituting metal or alloy are the same but have different compositions.

#### 1-1-2. Small Particles

In the present embodiment, the small particles **18** are magnetic particles. When the core **6** is manufactured using the small particles **18**, the core **6** has a higher packing density, and the inductor element **2** having a higher withstand voltage can be obtained.

The magnetic particles used for the small particles **18** are preferably metal magnetic particles or ferrite particles (more preferably, metal magnetic particles). Still more preferably, the magnetic particles used for the small particles **18** contain Fe.

Specifically, the metal magnetic particles containing Fe are pure iron, carbonyl Fe, Fe based alloy, Fe—Si based alloy, Fe—Al based alloy, Fe—Ni based alloy, Fe—Si—Al based alloy, Fe—Si—Cr based alloy, Fe—Co based alloy, Fe

based amorphous alloy, Fe based nanocrystalline alloy, etc. Preferably, the metal magnetic particles containing Fe are carbonyl Fe.

The ferrite particles are Mn—Zn, Ni—Cu—Zn, etc.

In the present embodiment, the small particles **18** may be structured by a plurality of small particles composed of the same material or a plurality of mixed small particles composed of different materials. For example, carbonyl Fe and multiple Fe—Si based alloy particles may be mixed and used for the small particles **18**.

In the present embodiment, the large particles **14** and the small particles **18** may be composed of the same material or different materials.

Preferably, each of the small particles **18** according to the present embodiment has a particle size of 2  $\mu\text{m}$  to 20  $\mu\text{m}$  (more preferably, 3  $\mu\text{m}$  to 7  $\mu\text{m}$ ).

Incidentally, the above-mentioned particle size excludes the cover part **28** of each of the small particles **14** mentioned below.

When the small particles **18** are structured by small particles composed of two or more types of different materials, the small particles **18** composed of a certain material and the small particles **18** composed of another material may have different particle sizes.

Incidentally, for example, the different materials mean that elements constituting metal or alloy are different from each other or that elements constituting metal or alloy are the same but have different compositions.

#### 1-1-3. Cover Part

In the present embodiment, a cover part may be formed on at least a part of each of the large particles **14** and the small particles **18**. In the manufacturing steps of the core **6**, the large particles **14** and the small particles **18** may contact with water. Thus, the cover part can prevent oxidation. If the large particles **14** or the small particles **18** are united with each other or the large particles **14** and the small particles **18** are united directly, magnetic characteristics (e.g., DC bias characteristic, withstand voltage characteristics) may be affected. Thus, grain boundaries are preferably formed by the cover part.

The cover part is composed of any materials of TEOS, MgO, glass, resin, phosphates (e.g., zinc phosphate, calcium phosphate, iron phosphate), or the like.

Incidentally, the cover parts **24** of the large particles **14** are preferably composed of TEOS. This makes it possible to maintain a high withstand voltage of the core.

Preferably, the cover parts **28** of the small particles **18** are preferably composed of MgO. This makes it possible to maintain high withstand voltage characteristics and a high corrosion resistance.

In the present embodiment, covering the large particle **14** and the small particles **18** with a material means that this material contacts with the large particle **14** and the small particles **18** and is fixed to cover this contact area.

The cover part covering the large particle **14** and the small particles **18** needs to at least partly cover the large particle **14** and the small particles **18**, but preferably covers the entire surface of each of the large particle **14** and the small particles **18**. Moreover, the cover part may continuously or intermittently cover each of the large particle **14** and the small particles **18**.

Incidentally, none of the large particles **14** and the small particles **18** may have the cover part. For example, 50% or more of the large particles **14** and 50% or more of the small particles **18** may have the cover part.

#### 1-1-4. Binder

Known resins can be used as a resin to be a binder constituting the core **6** (i.e., a resin to be the binder particles **16** of each of the composite particles **16**). Specifically, this resin is epoxy resin, phenol resin, polyimide resin, polyamide imide resin, silicone resin, melamine resin, urea resin, furan resin, alkyd resin, unsaturated polyester resin, diallyl phthalate resin, etc. and is preferably epoxy resin. The resin to be the binder particles **16** may be thermosetting resin or thermoplastic resin, but is preferably thermosetting resin.

#### 2. Method of Manufacturing Core

In the present embodiment, the core **6** is manufactured using the above-mentioned composite particles **12**. Thus, a method of manufacturing the composite particles **2** is initially explained, and a method of manufacturing the core **6** using the composite particles **12** is thereafter explained.

##### 2-1. Method of Manufacturing Composite Particles

A method of manufacturing the composite particles **12** according to the present embodiment includes: a step of preparing a first solution in which the large particles **14** are dispersed in a binder soluble solution in which a binder is dissolved; a step of preparing a second solution in which a binder insoluble solution is added to the first solution; and a step of drying the second solution.

First, the large particles **14** and the small particles **18** are prepared.

The large particles **14** and the small particles **18** may have a cover part. The cover part is formed on each of the large particles **14** and the small particles **18** by any known method. For example, the cover part can be formed by subjecting the large particles **14** and the small particles **18** to a wet processing.

Specifically, the large particles **14** and the small particles **18** are immersed into a solution in which compounds, their precursors, etc. to be constituting the cover part are dissolved, or this solution is sprayed against the large particles **14** and the small particles **18**. Then, the large particles **14** and the small particles **18** attached with this solution are subjected to a heat treatment. This makes it possible to form the cover part on each of the large particles **14** and the small particles **18**.

Next, the small particles **18** each having the cover part are attached on the large particles **14** each having the cover part in any manner. For example, the small particles **18** may be attached on the large particles **14** by electrostatic attraction, mechanochemical method, or synthetic deposition.

In order that the binder particles **16** are attached on each of the large particles **14** and located between two small particles **18a** and **18b** among the small particles **18** attached on each of the large particles **14**, the two small particles **18a** and **18b** need to be away from each other to some degree. From this point of view, the small particles **18** are preferably attached on each of the large particles **14** by electrostatic attraction. This is because, for electrostatic attraction, the large particles **14** and the small particles **18** are oppositely electrically charged and thereafter attracted, and the amount of the small particles **18** attached on each of the large particles **14** can thereby be controlled.

In the present embodiment, D90 of the small particles **18** is preferably smaller than D10 of the large particles **14**.

Here, D10 is a particle size of a particle whose cumulative frequency is 10%, counting from the smaller particle size.

D90 is a particle size of a particle whose cumulative frequency is 90%, counting from the smaller particle size.

Incidentally, particle size distribution (e.g., D10, D90) can be measured by particle size distribution measuring

machine, such as laser diffraction particle size distribution analyzer HELOS (Japan Laser Corporation).

The large particles **14** attached with the small particles **18** obtained in such a manner and a binder soluble solution are mixed.

Here, the binder soluble solution is a solution that is soluble to a binder insoluble solution and a binder to be added in the next step.

For example, when the binder to be added in the next step is a binder whose SP value is 10-15, such as epoxy resin (SP value: 10.9) and phenolic resin (SP value: 11.3), the binder soluble solution is a solvent whose SP value is 9.3-11, such as acetone (SP value: 9.9) and methyl ethyl ketone (SP value: 9.3).

The total concentration of the large particles **14** and the small particles **18** in the first solution is not limited (e.g., 10 mass % to 80 mass %). This makes it easier to attach the binder particles **16** onto each of the large particles **14** in the following steps.

Next, a first solution is prepared by adding the binder to the binder soluble solution containing the large particles **14** in any manner. For example, the binder can be added to the binder soluble solution containing the large particles **14** after binder solids are dissolved in the above-mentioned binder soluble solution.

In the first solution, the binder solid content is preferably 0.7 parts by mass to 4 parts by mass with respect to 100 parts by mass of the total of the large particles **14** and the small particles **18**. This makes it easier to attach the binder particles **16** onto each of the large particles **14** in the following steps.

Next, the second solution is prepared by adding a binder insoluble solution to the first solution.

Here, the binder insoluble solution is a solution that is insoluble to the binder added in the previous step and is soluble to the binder soluble solution.

For example, when the binder soluble solution employed in the above-mentioned step is a solvent whose SP value is 9.3-11 (e.g., acetone) and the binder added in the above-mentioned step is epoxy resin, the binder insoluble solution can be water (SP value: 23.4), ethanol (SP value: 12.7), or the like.

The second solution is prepared by adding the binder insoluble solution to the first solution, and the binder soluble solution is thereby dissolved in the binder insoluble solution. Thus, the binder dissolved in the binder soluble solution can be deposited as binder particles **16**. Due to the deposition of the binder as the binder particles **16**, the binder particles **16** can uniformly attach on each of the large particles **14** in the next step.

When the binder insoluble solution is added to the first solution, this mixture may be stirred in a lightly shaking manner.

The addition amount of the binder insoluble solution is not limited, but is preferably, for example, 15 parts by mass to 50 parts by mass with respect to 100 parts by mass of the binder soluble solution.

Then, an aggregation inhibitor is added to the second solution. The aggregation inhibitor is ethanol, IPA, or the like. This adjusts surface tension of the second solution and makes it possible to prevent the aggregation of the composite particles **12** in drying the second solution in the following step. In addition, the aggregation inhibitor can achieve a further higher consistency between pressing pressure and withstand voltage.

Preferably, 10 parts by mass to 50 parts by mass of the aggregation inhibitor are added with respect to 100 parts by mass of the binder soluble solution.

Next, the second solution added with the aggregation inhibitor is dried. This allows the deposited binder particles **16** to attach on each of the large particles **14** and makes it possible to obtain the composite particles **12** where the binder particles **16** are deposited on each of the large particles **14**. Preferably, each of the binder particles **16** according to the present embodiment has a particle size of 0.1  $\mu\text{m}$  to 10  $\mu\text{m}$  (more preferably, 1  $\mu\text{m}$  to 5  $\mu\text{m}$ ). This makes it possible to obtain the composite particles **12** where the binder particles **16** are dispersed to each of the large particles **14**.

The second solution added with the aggregation inhibitor is dried with any conditions and is dried, for example, for 30 minutes to 2 hours at (Tb-30)  $^{\circ}\text{C}$ . to Tb  $^{\circ}\text{C}$ ., where Tb is higher one of a boiling point of the binder soluble solution and a boiling point of the binder insoluble solution.

## 2-2. Method of Manufacturing Core

As shown in FIG. 1, the above-mentioned composite particles **12** and an air-core coil formed by winding a conductor (wire) **5** with a predetermined number are put into a die and pressed to obtain a green compact where the coil **5** is embedded. The composite particles **12** and the air-core coil are pressed in any manner (e.g., unidirectionally, isotropically with WIP, CIP, etc.), but are preferably pressed isotropically. This makes it possible to achieve rearrangement of the large particles **14** and the small particles **18** and densification of internal organization.

The obtained green compact is heated to obtain the core **6** having a predetermined shape where the large particles **14** and the small particles **18** are fixed, and the coil is embedded. Since the coil is embedded in the core **6**, the core **6** functions as a coil type electronic component like the inductor element **2**.

## 3. Summary of Present Embodiment

The present embodiment explained above is directed to the composite particle **12** including the large particle **14** having a particle size of 10  $\mu\text{m}$  to 50  $\mu\text{m}$  and the binder particles **16** attached on the large particle **14** and each having a particle size smaller than that of the large particle **14**.

The composite particles **12** have less characteristic variation after pressing. Specifically, a binder is uniformly present to the large particle **14** in the core **6** manufactured using the composite particles **12** according to the present embodiment.

When the core **6** is manufactured using the composite particles **12** according to the present embodiment, the consistency between pressing pressure and withstand voltage of the core **6** after pressing becomes high. Specifically, the higher pressing pressure is, the higher withstand voltage becomes. When the consistency between pressing pressure and withstand voltage of the core **6** after pressing becomes high, it is possible to obtain a desired withstand voltage based on pressing pressure and to stably adjust withstand voltage characteristics (product characteristics).

As a specific mode of the present embodiment, it is permissible to employ the composite particle **12** further including two or more small particles **18** attached on the large particle **14** and each having a particle size smaller than that of the large particle **14**, wherein the binder particles **16** are present on the large particle **14** and located between two small particles **18a** and **18b** among the small particles **18** attached on the large particle **14**.

When the core **6** is manufactured using the composite particles **12**, the packing density of the core **6** is increased, and withstand voltage characteristics are further improved.

As a specific mode of the present embodiment, it is permissible to employ the composite particles **12**, wherein the small particles **18** are magnetic particles.

The inductor element **2** can be manufactured with the core **6** using these composite particles **12**.

As a specific mode of the present embodiment, it is permissible to employ the composite particle **12**, wherein the large particle **14** is a magnetic particle.

The inductor element **2** can be manufactured with the core **6** using these composite particles **12**.

As a specific mode of the present embodiment, it is permissible to employ the composite particle **12**, wherein each of the binder particles **16** has a particle size smaller than that of the small particles **18**.

This composite particle **12** has further less characteristic variation after pressing.

When the core **6** is manufactured using the composite particles **12** according to the present embodiment, the consistency between pressing pressure and withstand voltage of the core **6** after pressing becomes further higher.

As a specific mode of the present embodiment, it is permissible to employ the composite particles **12**, wherein the binder particles **16** are deposited and attached on the large particle **14**.

Since the size and number of these binder particles **16** attached on the large particle **14** are controlled, the composite particle **12** has further less characteristic variation after pressing.

When the core **6** is manufactured using the composite particles **12** according to the present embodiment, the consistency between pressing pressure and withstand voltage of the core **6** after pressing becomes further higher.

The present embodiment is directed to the core **6** having a cross section or a surface on which the above-mentioned composite particle **12** is observed.

In the core **6** manufactured using the composite particles **12** according to the present embodiment, a binder is uniformly dispersed to each of the large particles **14**. Thus, the core **6** manufactured with the composite particles **12** according to the present embodiment has less characteristic variation after pressing.

When the core **6** is manufactured using the composite particles **12** according to the present embodiment, the consistency between pressing pressure and withstand voltage of the core **6** after pressing becomes high.

Moreover, the present embodiment is directed to the inductor element **2** including the above-mentioned core **6**.

In the core **6** manufactured using the composite particles **12** according to the present embodiment, the binder is uniformly present to the large particle **14**. Thus, the core **6** manufactured using the composite particles **12** according to the present embodiment has less characteristic variation after pressing. Thus, the inductor element **2** having less characteristic variation can be obtained using the core **6**.

When the core **6** is manufactured using the composite particles **12** according to the present embodiment, the consistency between pressing pressure and withstand voltage of the core **6** after pressing becomes high. Thus, using the core **6** makes it possible to obtain the inductor element **2** having stably adjust withstand voltage characteristics (product characteristics).

Moreover, the present embodiment is directed to a method of manufacturing composite particles. The method includes the steps of: preparing a first solution in which large particles

having a particle size of 10  $\mu\text{m}$  to 50  $\mu\text{m}$  are dispersed in a binder soluble solution in which a binder is dissolved; preparing a second solution in which a binder insoluble solution is added to the first solution; and drying the second solution, wherein the binder soluble solution is soluble to the binder and the binder insoluble solution, and wherein the binder insoluble solution is insoluble to the binder.

The composite particles **12** obtained by the method have less characteristic variation after pressing.

The consistency between pressing pressure and withstand voltage of the core **6** after pressing becomes high by manufacturing the core **6** using the composite particles **12** according to the present embodiment.

As a specific mode of the present embodiment, it is permissible to employ the method of manufacturing the composite particles **12**, wherein an aggregation inhibitor is added to the first solution in preparing the second solution.

This method adjusts surface tension of the second solution and makes it possible to prevent aggregation of the composite particles **12** in drying the second solution. Thus, the consistency between pressing pressure and withstand voltage of the core **6** after pressing becomes high by manufacturing the core **6** using the composite particles **12** according to the present embodiment.

As a specific mode of the present embodiment, it is permissible to employ the method of manufacturing the composite particles **12**, wherein a small particle **18** having a particle size smaller than that of each of the large particles **14** is attached on each of the large particles **14** in the first solution.

This method increases the packing density of the core **6** and further improves withstand voltage characteristics.

Moreover, the present embodiment is directed to composite particles **12** obtained by the above-mentioned method.

The composite particles **12** obtained by the method have less characteristic variation after pressing.

The consistency between pressing pressure and withstand voltage of the core **6** after pressing becomes high by manufacturing the core **6** using the composite particles **12** according to the present embodiment.

Hereinbefore, an embodiment of the present invention is explained, but the present invention is not limited to the above-mentioned embodiment and may be modified in various embodiments within the scope of the present invention.

For example, the inductor element **2** has a structure where an air-core coil formed by winding the conductor **5** is embedded in the core **6** having a predetermined shape shown in FIG. 1, but may have any other structure as long as the conductor is wound on the core having a predetermined shape.

For example, the core may have a FT shape, an ET shape, an EI shape, a UU shape, an EE shape, an EER shape, a UI shape, a drum shape, a toroidal shape, a pot shape, a cup shape, or the like.

For example, the composite particles **12** according to the above-mentioned embodiment contain the small particles **18**, but the small particles **18** may not necessarily be contained in the composite particles **12**.

In this case, the number of binder particles **16** attached on each of the large particles **14** is preferably one or more (more preferably, six or more). This makes it possible to obtain the composite particles **12** where the binder particles **16** are dispersed to each of the large particles **14**.

In this case, the particle size of each of the binder particles **16** attached on each of the large particles **14** is smaller than that of each of the large particles **14** and is preferably 0.1  $\mu\text{m}$

## 11

to 10  $\mu\text{m}$  (more preferably, 1  $\mu\text{m}$  to 5  $\mu\text{m}$ ). This makes it possible to obtain the composite particles **12** where the binder particles **16** are dispersed to each of the large particles **14**.

In the above-mentioned embodiment, each of the large particles **14** has the cover part **24**, and each of the small particles **18** has the cover part **28**. However, the large particles **14** and the small particles **18** may have no cover part.

In the above-mentioned embodiment, the first solution is prepared by adding a binder to the binder soluble solution containing the large particles **14**, but the first solution may be formed by adding the large particles **14** to the binder soluble solution containing a binder.

In the above-mentioned embodiment, an aggregation inhibitor is added to the second solution after it is formed, but the aggregation inhibitor may be added in preparing the second solution. That is, the second solution may be prepared by adding the binder insoluble solution after the aggregation inhibitor is added to the first solution, or the second solution may be prepared by simultaneously adding the aggregation inhibitor and the binder insoluble solution to the first solution.

In the above-mentioned embodiment, the composite particles **12** used for the core **6** are explained. However, the composite particles **12** according to the present invention are used not only for the core **6**, but for products containing particles and binder, such as paste products (e.g., dielectric paste, electrode paste), bonded magnets formed by mixing magnetic powder and binder, and polymer solid electrolyte formed by mixing lithium ion conductive solid electrolyte material and binder. In addition, the composite particles **12** according to the present invention can be used for magnetic shield sheets.

When the composite particles **12** according to the present invention is used for dielectric paste, the large particles **14** are composed of barium titanate, calcium titanate, strontium titanate, etc., and the small particles **18** are composed of silicon, rare earth element, alkaline earth metal, etc.

When the composite particles **12** according to the present invention are used for electrode paste, the large particles **14** are composed of Ni, Cu, Ag, Au, their alloys, etc.

Moreover, the large particles **14** are composed of any material. The large particles **14** may be composed of magnetic particles as explained in the above-mentioned embodiment or ceramics (e.g., barium titanate), Ni, etc. as mentioned above. Besides, the large particles **14** may be composed of alumina, polymer (epoxy, PPS, PES, PS, PMMA, Pa), etc.

The small particles **18** are also composed of any material. The small particles **18** may be composed of magnetic particles as explained in the above-mentioned embodiment or silicon etc. as mentioned above. Besides, the small particles **18** may be composed of alumina, ceramics (e.g., barium titanate), polymer (epoxy, PPS, PES, PS, PMMA, Pa), etc.

## EXAMPLES

Hereinafter, the present invention is explained in more detail with Examples, but is not limited thereto.

## Example 1

Large particles **14** attached with small particles **18** by electrostatic attraction were prepared.

## 12

The material of the large particles **14** was Fe—Si based alloy. The average particle size of the large particles **14** was 30  $\mu\text{m}$ . A cover part **24** was formed on each of the large particles **14**. The material of the cover parts **24** of the large particles **14** was TEOS.

The material of the small particles **18** was carbonyl Fe. The average particle size of the small particles **18** was 4.0  $\mu\text{m}$ . A cover part **28** was formed on each of the small particles **18**. The material of the cover parts **28** of the small particles **18** was MgO.

Next, an acetone was prepared as a binder soluble solution. The large particles **14** attached with the small particles **18** and the acetone were mixed and dispersed so that the total concentration of the large particles **14** and the small particles **18** would be 33 mass %.

Then, a binder solution (binder solid: epoxy resin, binder solid concentration: 33 mass %) was added to the liquid mixture to prepare a first solution. In the first solution, the binder solid content was 2 parts by weight to 100 parts by weight of the total of the large particles **14** and the small particles **18**.

Next, a water was prepared as a binder insoluble solution. 7.5 parts by mass of the water were added to 100 parts by mass of the acetone contained in the first solution to prepare a second solution.

Then, an ethanol (aggregation inhibitor) was added to the second solution. 7.5 parts by mass of the ethanol were added to 100 parts by mass of the acetone.

Next, the second solution added with the ethanol was dried at 70° C. to 100° C. for one hour to obtain composite particles **12**.

The composite particles **12** obtained in such a manner were filled in a predetermined rectangular-parallelepiped die where a predetermined insertion member was disposed. The predetermined insertion member was a conductor **5** having a winding part **4** (inner diameter: 4 mm, height: 3 mm). The die was set at 80° C. and pressed unidirectionally at 400 MPa (pressing pressure) to obtain a green compact of a core **6**. The green compact of the manufactured core **6** was subjected to a heat hardening treatment at 200° C. for five hours in the air to obtain a rectangular-parallelepiped core **6** (length: 7 mm, width: 7 mm, height: 5.4 mm).

The number of cores **6** manufactured was three.

Incidentally, it was confirmed that none of the particle size of each of the large particles **14**, the particle size of each of the small particles **18**, the mixing ratio of the large particles **14**, the mixing ratio of the small particles **18**, and the mixing ratio of the binder **16** changed in the above-mentioned manufacturing steps.

Voltage was applied between terminal electrodes of the rectangular-parallelepiped core **6** using a DC Power Supply manufactured by KEYSIGHT and an LCR meter, and a voltage when 0.5 mA (electric current) flowed was determined to be a withstand voltage. This measurement was carried out for each of the three rectangular-parallelepiped cores **6**.

## Examples 2-4

60 Except for changing the pressing pressure as described in Table 1, rectangular-parallelepiped cores **6** were obtained to measure a withstand voltage as with Example 1.

## Comparative Example 1

65 Large particles **14** attached with small particles **18** by electrostatic attraction were prepared. The material and the

## 13

average particle size of the large particles **14** and the small particles **18** and the materials of the cover parts were the same as those of Example 1.

The large particles **14** attached with the small particles **18** and an epoxy resin solution (solvent:acetone) were mixed. The solid content of the epoxy resin was 2 parts by mass to 100 parts by mass of the total of the large particles **14** and the small particles **18**. After the mixing, the acetone was volatilized to obtain granules.

Except for using the granules obtained in such a manner, a rectangular-parallelepiped magnetic material of Comparative Example 1 was obtained to measure a withstand voltage as with Example 1. The results are shown in Table 2.

## Comparative Examples 2-4

Except for changing the pressing pressure as described in Table 2, rectangular-parallelepiped cores **6** of Comparative Examples 2-4 were obtained to measure a withstand voltage as with Comparative Example 1. The results are shown in Table 2.

TABLE 1

| Sample No. | Pressing Pressure<br>[MPa] | Withstand Voltage<br>[kV] |
|------------|----------------------------|---------------------------|
| Example 1  | 400                        | 0.47                      |
|            |                            | 0.46                      |
|            |                            | 0.47                      |
| Example 2  | 600                        | 0.52                      |
|            |                            | 0.52                      |
|            |                            | 0.52                      |
| Example 3  | 800                        | 0.55                      |
|            |                            | 0.52                      |
|            |                            | 0.54                      |
| Example 4  | 1000                       | 0.63                      |
|            |                            | 0.61                      |
|            |                            | 0.62                      |

TABLE 2

| Sample No.            | Pressing Pressure<br>[MPa] | Withstand Voltage<br>[kV] |
|-----------------------|----------------------------|---------------------------|
| Comparative Example 1 | 400                        | 0.62                      |
|                       |                            | 0.59                      |
|                       |                            | 0.61                      |
| Comparative Example 2 | 600                        | 0.45                      |
|                       |                            | 0.47                      |
|                       |                            | 0.46                      |
| Comparative Example 3 | 800                        | 0.38                      |
|                       |                            | 0.46                      |
|                       |                            | 0.42                      |
| Comparative Example 4 | 1000                       | 0.47                      |
|                       |                            | 0.35                      |
|                       |                            | 0.42                      |

FIG. 5 is a graph made based on Table 1 and Table 2. In FIG. 5, the X-axis means withstand voltage, and the Y-axis means pressing pressure. "Examples" corresponds to Examples 1-4, and "Comparative Examples" corresponds to Comparative Examples 1-4.

FIG. 5 shows that the cores manufactured using the predetermined composite particles (Examples) had less variation in withstand voltage in the samples even though the pressing pressure was high compared to the cores manufactured using the granules prepared by the method of Comparative Examples (hereinafter, referred to as "comparative-example granules"). That is, FIG. 5 shows that the cores manufactured using the predetermined composite par-

## 14

ticles (Examples) had less variation in withstand voltage after pressing compared to the cores manufactured using the comparative-example granules.

Moreover, the withstand voltage was further improved as the pressing pressure was higher in the cores manufactured using the predetermined composite particles (Examples). This confirms that Examples had a high consistency between pressing pressure and withstand voltage. This also confirms that Examples had a higher consistency between pressing pressure and withstand voltage compared to the cores manufactured using the comparative-example granules.

The reason why Examples had less variation in withstand voltage after pressing and a high consistency between pressing pressure and withstand voltage is probably that Examples used the predetermined composite particles of the present invention. In the composite particles of the present invention, as shown in FIG. 2 and FIG. 3, the binder was present as binder particles, and the binder particles were uniformly dispersed and attached on each of the large particles. Thus, it is conceivable that the large particles, the small particles, and the binder particles were kept uniformly dispersed even though the composite particles were put into the die and pressed. Then, it is conceivable that the dispersion state of the large particles, the small particles, and the binder particles contributed to the effects of less characteristic variation after pressing and high consistency between pressing pressure and withstand voltage.

On the other hand, as shown in FIG. 4, it is conceivable that the binder was unevenly attached on each of the large particles in Comparative Examples. Thus, it is conceivable that Comparative Examples were inferior to Examples in terms of characteristic variation after pressing and consistency between pressing pressure and withstand voltage.

## Example 5

Except for changing the pressing pressure to 600 MPa and the pressing temperature to 50° C., rectangular-parallelepiped cores **6** were obtained to measure a withstand voltage as with Example 1. The results are shown in Table 3. In Example 5, a toroidal core was obtained in addition to the rectangular-parallelepiped cores **6**, and an initial permeability was also measured. The results are shown in Table 3. The toroidal core was obtained in the following manner. The initial permeability was measured in the following manner.

Composite particles **2** obtained similarly to Example 1 were filled in a predetermined toroidal die and pressed at 400 MPa (pressing pressure) to obtain a green compact of the core. The green compact of the manufactured core was subjected to a heat hardening treatment at 200° C. for five hours in the air to obtain a toroidal core (outer diameter: 15 mm, inner diameter: 9 mm, thickness: 0.7 mm).

The toroidal core was wound by a coil in 32 turns. Then, an initial permeability  $\mu_i$  was measured by an LCR meter (LCR428A manufactured by HP).

## Example 6

Except for changing the temperature of the die at pressing to 70° C., rectangular-parallelepiped cores and a toroidal core were obtained to measure a withstand voltage and an initial permeability were measured as with Example 5. The results are shown in Table 3.

## Example 7

Except for obtaining green compacts of rectangular-parallelepiped cores and a toroidal core by pressing the cores at

## 15

200 MPa (pressing pressure) and 80° C. with Warm Isostatic Press (WIP), the rectangular-parallelepiped cores and the toroidal core were obtained to measure a withstand voltage and an initial permeability as with Example 6. The results are shown in Table 3.

TABLE 3

| Sample No. | Pressing Pressure<br>[MPa] | Withstand Voltage<br>[V] | Initial<br>Permeability |
|------------|----------------------------|--------------------------|-------------------------|
| Example 5  | 600                        | 0.07~0.4                 | 25                      |
| Example 6  | 600                        | 0.12~0.50                | 26.5~30                 |
| Example 7  | 200                        | 0.96~2.13                | 25~29.5                 |

Table 3 shows that the initial permeability was substantially the same between the unidirectional pressing (Examples 5 and 6) and the isotropical pressing (Example 7).

Table 3 also shows that the withstand voltage in the isotropical pressing (Example 7) was higher than that in the unidirectional pressing (Examples 5 and 6). This is probably because the rearrangement of the large particles and the small particles and the densification of internal organization were achieved in the isotropical pressing (WIP) (Example 7).

DESCRIPTION OF THE REFERENCE  
NUMERICAL

- 2 . . . inductor element
  - 4 . . . winding part
  - 5 . . . conductor
  - 6 . . . core
  - 12 . . . composite particle
  - 14 . . . large particle
  - 16 . . . binder particle
  - 18, 18a, 18b . . . small particle
  - 24 . . . cover part of large metal magnetic particle
  - 28a, 28b . . . cover part of small metal magnetic particle
  - 38a, 38b . . . connection point between small metal magnetic particle and large metal magnetic particle
  - 46 . . . binder
- What is claimed is:
1. A composite particle comprising:  
a large particle having a particle size of 10  $\mu\text{m}$  to 50  $\mu\text{m}$ ;  
binder particles attached on the large particle and each  
having a particle size smaller than that of the large  
particle, and  
two or more small particles attached on the large particle  
and each having a particle size smaller than that of the  
large particle,

## 16

wherein at least one of the binder particles is attached on  
the large particle and located between two small par-  
ticles among the two or more small particles attached  
on the large particle,

- 5 wherein the large particle is a magnetic particle,  
wherein the binder particles comprise thermosetting resin  
or thermoplastic resin, and  
wherein the small particles are magnetic particles.

- 10 2. The composite particle according to claim 1, wherein  
each of the binder particles has a particle size smaller than  
that of the small particles.

- 15 3. A core having a cross section or a surface on which the  
composite particle according to claim 1 is observed.

- 15 4. An inductor element comprising the core according to  
claim 3.

- 20 5. The composite particle according to claim 1, wherein  
each of (dL/dS), (dL/dB), and (dS/dB) satisfies the following  
relation, where dL is a particle size of the large particle, dS  
is a particle size of the small particle, and dB is a particle size  
of the binder particle:

$$1 < (dL/dS) \leq 25,$$

$$1 < (dL/dB) \leq 500, \text{ and}$$

$$0.6 \leq (dS/dB) \leq 200.$$

- 25 6. The composite particle according to claim 5, wherein  
1.4  $\leq (dL/dS) \leq 8.3$ ,

$$2 \leq (dL/dB) \leq 25, \text{ and}$$

$$1.0 \leq (dS/dB) \leq 7.0.$$

- 30 7. The composite particle according to claim 1, wherein at  
least a part of each of the large particles has a cover part  
formed thereon.

- 35 8. The composite particle according to claim 7, wherein  
the cover part is composed of TEOS, MgO, glass, resin, or  
a phosphate.

- 40 9. The composite particle according to claim 7, wherein at  
least a part of each of the small particles has a cover part  
formed thereon.

- 45 10. The composite particle according to claim 9, wherein  
the cover part of the large particle is composed of TEOS, and  
the cover part of the small particle is composed of MgO.

- 50 11. The composite particle according to claim 1, wherein  
at least a part of each of the small particles has a cover part  
formed thereon.

- 55 12. The composite particle according to claim 11, wherein  
the cover part is composed of MgO.

\* \* \* \* \*